# EUROPEAN PATENT APPLICATION

(11) **EP 2 447 350 A1**
(43) Date of publication of application: **02.05.2012**
(21) Application number: 10189527.4
(22) Date of filing: 29.10.2010
(51) Int. Cl.: C11D 17/00, C11D 3/395, C11D 3/37, C11D 3/39

(54) **Bleach coparticle**

(71) Applicant: The Procter & Gamble Company, Cincinnati, OH 45202 (US)
(72) Inventor: Somerville Roberts, Nigel Patrick, Newcastle upon Tyne, NE20 9AU (GB); Parmley, David James, Tyne and Wear, NE9 5BH (GB); Castro, Jerome Macaisa, Newcastle upon Tyne, NE12 9PG (GB); Guida, Vincenzo,, Rome 00142, (IT); Mort, Paul R., Cincinnati, OH42515 (US)
(74) Representative: Vercruysse, Nicolas

(57) **Abstract**

Layered particles that contain a source of hydrogen peroxide, a binder material, and a bleach activator are disclosed. The disclosed layered particles have improved properties and are useful, for example, for incorporation into granular detergents. A method of improving the stability of a source of hydrogen peroxide is also disclosed.

## Description

### FIELD OF THE INVENTION

Layered particles, compositions comprising such particles as well as methods of making and using such particles and compositions, are disclosed. A method of improving the stability of a source of hydrogen peroxide is also disclosed.

### BACKGROUND OF THE INVENTION

Inorganic peroxide compounds exert a bleaching effect during the laundering process via release of hydrogen peroxide upon contact with water. This effect may be enhanced in the presence of bleaching activators such as sodium-nonaolyloxy benzene sulfonate (NOBS), tetraacetyl ethylene diamine (TAED) and the like. These bleaching systems are often used in granule detergent compositions, the hydrogen peroxide source being agents such as sodium percarbonate and perborate. Such systems, however, suffer from the problem of being unstable over time when mixed with many detergent products. For example, the presence of water may lead to an exothermic degradation of the system.

Another issue is that the efficiency of the bleaching systems in the wash is reduced by the presence of the enzyme catalase in soiled laundry. Catalase is extremely efficient at degrading hydrogen peroxide and even the minute quantities present in laundry items as a result of contact with human skin can degrade a major part of the hydrogen peroxide used in wash systems. To overcome this problem, hydrogen peroxide sources such as sodium percarbonate are generally added in excess molar quantities - often several times the stoichiometric quantities needed for the reaction with the bleach activator. Thus, there is also a need for bleaching systems that effectively use bleaching raw materials, for example, hydrogen peroxide sources.

One way to minimize the issue of degradation of hydrogen peroxide by catalase is to closely co-locate the bleach activator and the peroxide source, e.g. percarbonate. Combining commonly used bleach activators with alkaline percarbonate is problematic, however, due to the fact that these bleach activators (TAED and NOBS) tend to degrade in alkaline environments. Thus, closely combining these bleach activators with alkaline percarbonate generally causes degradation of the bleach activator on storage. Attempts have been made to create particles comprising percarbonate and bleach activator to increase stability these systems using binders and other additives which coat the source of hydrogen peroxide. (*See, e.g.,* WO 2007/127641, published also as US20070252107A1.) However, such approaches either cannot be conveniently used in a continuous process, and/or do not provide particles having suitable release profiles and/or do not have sufficient stability on storage.

Accordingly, there is a need for particles comprising hydrogen peroxide bleaching systems and optionally bleach activators that have good storage stability, suitable solubility in laundering processes, and/or improved hydrogen peroxide source use efficiency. The instant disclosure addresses one or more of the aforementioned needs.

### SUMMARY OF THE INVENTION

Layered particles, compositions comprising such particles as well as methods of making and using such particles and compositions, are disclosed. A method of improving the stability of a source of hydrogen peroxide is also disclosed.

### DETAILED DESCRIPTION OF THE INVENTION

As used herein, articles such as "a" and "an" when used in a claim, are understood to mean one or more of what is claimed or described.

As used herein, the term "additive" means a composition or material that may be used separately from (but including before, after, or simultaneously with) the detergent during a laundering process to impart a benefit to the treated textile.

As used herein, the term "core," as applied to a source of hydrogen peroxide such as percarbonate, includes the active agent itself in addition to any coating applied by the manufacturer.

As used herein, the term "gelling agent" means a material capable of forming a gel upon contact with water.

"Gel" as defined herein refers to a transparent or translucent liquid having a viscosity of greater than about 2000 mPa*s at 25°C and at a shear rate of 20 sec-¹. In some embodiments, the viscosity of the gel may be in the range of from about 3000 to about 10,000 mPa*s at 25°C at a shear rate of 20 sec-¹ and greater than about 5000 mPa*s at 25°C at a shear rate of 0.1 sec⁻¹.

As used herein, the terms "include", "includes" and "including" are meant to be non-limiting.

As used herein, the term "layer" means a partial or complete coating of a layering material built up on a particle's surface or on a coating covering at least a portion of said surface.

As used herein, "particle size" refers to the diameter of the particle at its longest axis.

As used herein, the term "mean particle size" means the mid-point of the size distribution of the particles made herein, determined according to the methods disclosed herein.

As used herein, the term "solvent" is meant to connote a liquid portion that may be added to one or more components described herein. The term "solvent" is not intended to require that the solvent material be capable of actually dissolving all of the components to which it is added. Exemplary solvents include alkylene glycol mono lower alkyl ethers, propylene glycols, ethoxylated or propoxylated ethylene or propylene, glycerol esters, glycerol triacetate, lower molecular weight polyethylene glycols, lower molecular weight methyl esters and amides, and the like.

As used herein, "substantially free of" a component means that no amount of that component is deliberately incorporated into the composition.

Unless otherwise noted, all component or composition levels are in reference to the active portion of that component or composition, and are exclusive of impurities, for example, residual solvents or by-products, which may be present in commercially available sources of such components or compositions.

All percentages and ratios are calculated by weight unless otherwise indicated. All percentages and ratios are calculated based on the total composition unless otherwise indicated.

It should be understood that every maximum numerical limitation given throughout this specification includes every lower numerical limitation, as if such lower numerical limitations were expressly written herein. Every minimum numerical limitation given throughout this specification will include every higher numerical limitation, as if such higher numerical limitations were expressly written herein. Every numerical range given throughout this specification will include every narrower numerical range that falls within such broader numerical range, as if such narrower numerical ranges were all expressly written herein. Applicants recognized that it is possible to make a co-particle of a peroxide source, such as percarbonate, and bleach activator that overcomes one or more of the problems described above. The disclosed compositions comprise, in general, a layered particle where the TAED or other bleach activator is layered around a percarbonate (or other hydrogen peroxide source) particle to form a substantially continuous coating. Applicants recognized that the stability of the bleach activator in particular can be improved during storage by varying the ratio of the bleach activator to the percarbonate, with particle storage stability increasing as the ratio of bleach activator to percarbonate is increased. Without being bound by theory, the increase in storage stability is believed to be due to the thickening of the coating layer of bleach activator around the core particle arising from the increase in the activator portion. This in turn results in the proportion of the bleach activator in close contact with the surface of the percarbonate being reduced. In another aspect, the bleach activator may be diluted in the layering powder to form a thicker, but diluted layer, which will also reduce the proportion of bleach activator in close proximity with the surface of the bleach activator. Without being bound by theory, Applicants believe that the thicker the layer provided, the greater the barrier to moisture ingress to the percarbonate surface. Reduced moisture ingress, in turn, is believed to improve overall stability of the layered particle.

Applicants have further recognized that, by selecting the proper binder, layered particles comprising a source of hydrogen peroxide and a bleaching activator can be formed, such that the layered particles have improved storage stability and a favorable dissolution profile. In one aspect, the layered particles disclosed herein allow for the co-localization of bleach activators and the source of hydrogen peroxide, thus allowing for improved efficiency in addition to improved stability. In another aspect, the layered particles are impermeable or have decreased permeability to catalase under wash conditions.

Applicants have also recognized that the use of a specific binder comprising at least 10% by weight of the binder of material absorbing more than 10% water by weight of said binder over a relative humidity of 60% at 25°C could increase the thermal stability of the system. Without being bound by theory, such a binder has the ability to soak up part of the water, thus limiting the amount of water in direct contact with moisture sensitive material.

In one aspect, a layered particle comprising a core and a layer, said core comprising a source of hydrogen peroxide and said layer comprising a binder and a bleach activator, wherein the weight ratio of said source of hydrogen peroxide to said bleach activator may be from about 5:1 to about 1.1:1, or from about 4:1 to about 1.5:1, or about 2:1 is disclosed.

In one aspect, the layered particle may have an average diameter of from about 600 µm to 2000 µm, or from about 800 µm to about 1000 µm. In one aspect, the layer may have a thickness of from about 25 µm to about 150 µm, or from about 40 µm to about 100 µm.

Binder - The binder may represent, based on total layered particle weight, from about 2% to about 20%, or from about 4% to about 15%, or about 6% to about 10%, or from about 7% to about 8% of said layered particle. The binder may comprise, based on total layered particle weight, from about 0.001% to about 5%, or from about 0.5% to about 3%, or about 1% to about 2% water. In one aspect, the binder may be substantially free of water. In one aspect, the binder may be capable of absorbing from about 0.1% to about 20%, or from about 1% to about 15%, or from about 2% to about 10% water by weight of said binder over a relative humidity of 80% at 32°C. In one aspect, the binder may have a viscosity of from about 200 to about 20,000, or from about 500 to about 7,000, or from about 1,000 to about 2,000 centipoise at a shear rate of 25 sec⁻¹ at 25°C.

The binder comprise at least 10% by weight of the binder of material absorbing more than 10% water by weight of said binder over a relative humidity of 60% at 25°C. This can be measured as in the test method below "determination of water intake".

In particular, the binder may comprise at least 20% or 30% or 50% or at least 70% or 90% by weight of the binder of material absorbing more than 10% water by weight of said binder over a relative humidity of 60% at 25°C

The binder may comprise at least 20% or 30% or 50% or at least 70% or 90% by weight of the binder of material absorbing more than 20% water by weight of said binder over a relative humidity of 60% at 25°C

The binder may comprise at least 20% or 30% or 50% or at least 70% or 90% by weight of the binder of material absorbing more than 30% water by weight of said binder over a relative humidity of 60% at 25°C

The binder may comprise at least 20% or 30% or 50% or at least 70% or 90% by weight of the binder of material absorbing more than 40% water by weight of said binder over a relative humidity of 60% at 25°C

The binder may comprise, based on total binder weight, from about 10% or 20% or 40% or 60% or 80% to 100%, or 99% or 95% by weight of a polymeric material. The polymeric material may comprise maleic acrylic copolymer, polyvinylpyrolidone, polyethylene glycol (to be completed) or mixtures thereof.

The binder may comprise, based on total binder weight, from about 10% or 20% or 40% or 50% of cationic surfactant.

The source of hydrogen peroxide may comprise a per-compound. The sources of hydrogen peroxide may include sodium perborate in mono-hydrate or tetra-hydrate form or mixtures thereof, sodium percarbonate, and combinations thereof. In one aspect, the source of hydrogen peroxide may be sodium percarbonate. The sodium percarbonate may be in the form of a coated percarbonate particle.

The bleach activator may comprise a material selected from the group consisting of bleach activators such as tetraacetyl ethylene diamine; oxybenzene sulphonate bleach activators such as nonanoyl oxybenzene sulphonate; caprolactam bleach activators; imide bleach activators such as N-nonanoyl-N-methyl acetamide; preformed peracids such as N,N-pthaloylamino peroxycaproic acid, nonylamido peroxyadipic acid, or dibenzoyl peroxide; decanoyloxybenzenecarboxylic acid (DOBA); and combinations thereof. In one aspect, the bleach activator may be nonanoyl oxybenzene sulphonate, tetraacetyl ethylene diamine, and combinations thereof. In one aspect, the bleach activator may be tetraacetyl ethylene diamine. Non limiting examples of bleach activators are disclosed in, for example, USPNs 4,915,854 and 4,412,934.

In one aspect, the layered particle may comprise a dusting powder that may comprise a material selected from the group consisting of silicas; zeolites; amorphous aluminosilicates; clays; starches; celluloses; water soluble salts, such as an inorganic salt selected from the group consisting of, sodium chloride, sodium sulphate, magnesium sulphate, and salts and mixtures thereof; polysaccharides including sugars; and combinations thereof.

### Additives

The layer may comprise an additive selected from the group consisting of acidic materials, moisture sinks; gelling agents; antioxidants; organic catalysts and combinations thereof.

In one aspect, the additive may comprise an acidic material having a pKa of from about 3 to about 7, or about 5. In one aspect, the acidic material may be ascorbic acid.

In one aspect, the additive may comprise a moisture sink that may be selected from the group consisting of crosslinked polyacrylates; sodium salts of maleic/acrylic copolymers; magnesium sulfate; and combinations thereof.

In one aspect, the additive may comprise a gelling agent that may be selected from the group consisting of a cellulose including methylcellulose and CMC; alginate and derivatives thereof; starches; polyvinyl alcohols; polyethylene oxide; polyvinylpyrolidone; polysaccharides including chitosan and/or natural gums including carrageenan, xantham gum, guar gum, locust bean gum, and combinations thereof; polyacrylates including cross-linked polyacrylates; alcohol ethoxylates; lignosulfonates; surfactants and mixtures thereof; powdered anionic surfactants; and combinations thereof.

In one aspect, the additive may comprise an antioxidant that may be selected from the group consisting of phenolic antioxidants; amine antioxidants; alkylated phenols; hindered phenolic compounds; benzofuran or benzopyran; alpha-tocopherol, beta-tocopherol, gamma-tocopherol, delta-tocopherol, and derivatives thereof; 6-hydroxy-2,5,7,8-tetra-methylchroman-2-carboxylic acid; ascorbic acid and its salts; butylated hydroxy benzoic acids and their salts; gallic acid and its alkyl esters; uric acid and its salts and alkyl esters; sorbic acid and its salts; amines; sulfhydryl compounds; dihydroxy fumaric acid and its salts; and combinations thereof, 2,6-di-tertbutylphenol; 2,6-di-tert-butyl-4-methylphenol; mixtures of 2 and 3-tert-butyl-4-methoxyphenol; propyl gallate; tert-butylhydroquinone; benzoic acid derivatives such as methoxy benzoic acid; methylbenzoic acid; dichloro benzoic acid; dimethyl benzoic acid; 5-hydroxy-2,2,4,6,7-pentamethyl-2,3-dihydro-1-benzofuran-3-one; 5-hydroxy-3-methylene-2,2,4,6, 7-pentamethyl-2,3-dihydro-benzofuran; 5-benzyloxy-3-hydroxymethyl-2,2,4,6,7-pentamethyl-2,3-dihydro-1-benzofura- n, 3-hydroxymethyl-5-methoxy-2,2,4,6,7-pentamethyl-2,3-dihydro-1-benzofura- n; ascorbic acid; 1,2-dihydro-6-ethoxy-2,2,4-trimethylchinolin, and combinations thereof; 2,6-di-tert-butyl hydroxy toluene; alpha-tocopherol; hydroquinone, 2,2,4-trimethyl-1,2-dihydroquinoline; 2,6-di-tert-butyl hydroquinone; 2-tert-butyl hydroquinone; tert-butyl-hydroxy anisole; lignosulphonic acid and salts thereof; benzoic acid and derivatives thereof; trimethoxy benzoic acid; toluic acid; catechol; t-butyl catechol; benzylamine; amine alcohols; 1,1,3-tris(2-methyl-4-hydroxy-5-t-butylphenyl) butane; N-propyl-gallate or mixtures thereof; or di-tert-butyl hydroxy toluene.

In one aspect, the additive may comprise an organic catalyst that may be selected from the group consisting of iminium cations and polyions; iminium zwitterions; modified amines; modified amine oxides; N-sulphonyl imines; N-phosphonyl imines; N-acyl imines; thiadiazole dioxides; perfluoroimines; cyclic sugar ketones; and combinations thereof; or an organic catalyst selected from the group consisting of 2-[3-[(2-hexyldodecyl)oxy]-2-(sulfooxy)propyl]-3,4-dihydroisoquinolinium, inner salt; 3,4-dihydro-2-[3-[(2-pentylundecyl)oxy]-2-(sulfooxy)propyl]isoquinolinium, inner salt; 2-[3-[(2-butyldecyl)oxy]-2-(sulfooxy)propyl]-3,4-dihydroisoquinolinium, inner salt; 3,4-dihydro-2-[3-(octadecyloxy)-2-(sulfooxy)propyl]isoquinolinium, inner salt; 2-[3-(hexadecyloxy)-2-(sulfooxy)propyl]-3,4-dihydroisoquinolinium, inner salt; 3,4-dihydro-2-[2-(sulfooxy)-3-(tetradecyloxy)propyl]isoquinolinium, inner salt; 2-[3-(dodecyloxy)-2-(sulfooxy)propyl]-3,4-dihydroisoquinolinium, inner salt; 2-[3-[(3-hexyldecyl)oxy]-2-(sulfooxy)propyl]-3,4-dihydroisoquinolinium, inner salt; 3,4-dihydro-2-[3-[(2-pentylnonyl)oxy]-2-(sulfooxy)propyl]isoquinolinium, inner salt; 3,4-dihydro-2-[3-[(2-propylheptyl)oxy]-2-(sulfooxy)propyl]isoquinolinium, inner salt; 2-[3-[(2-butyloctyl)oxy]-2-(sulfooxy)propyl]-3,4-dihydroisoquinolinium, inner salt; 2-[3-(decyloxy)-2-(sulfooxy)propyl]-3,4-dihydroisoquinolinium, inner salt; 3,4-dihydro-2-[3-(octyloxy)-2-(sulfooxy)propyl]isoquinolinium, inner salt; 2-[3-[(2-ethylhexyl)oxy]-2-(sulfooxy)propyl]-3,4-dihydroisoquinolinium, inner salt or mixtures thereof; or 2-[3-[(2-butyloctyl)oxy]-2-(sulfooxy)propyl]-3,4-dihydroisoquinolinium, inner salt.

In one aspect, the layered particle may be substantially free of fatty acids, fatty acid polyol esters, polyglycols, and fatty alcohol oxalkylates.

### Method of Improving Stability of a Source of Hydrogen Peroxide

In another aspect, a method of improving the stability of a source of hydrogen peroxide, such as a percarbonate particle is disclosed. In this aspect, the method may comprise the step of providing a layer that may comprise a binder comprising at least 10% by weight of the binder of material absorbing more than 10% water by weight of said binder over a relative humidity of 60% at 25°C., wherein said binder may comprise from about 0.001% to about 5%, or from about 0.5% to about 3%, or about 1% to about 2% water, or is substantially free of water; wherein said layer substantially coats said source of hydrogen peroxide.

Preferably, the layered particle is dried. For example the particle may be dried in a fluid bed drier. For example at a temperature of above 60°C or 80°C or 100°C. This insures that the level of water in the particle, and in particular in the binder is low. Accordingly, the amount of water that the binder can soak up is increased and the thermal stability of the particle is ameliorated.

### TEST METHODS

Binder Component Viscosity Test - This test method must be used to determine binder component viscosity. Viscosity is determined using a Paar Physica UDS 200 using a Z3 cup and spindle at 25°C in accordance with the manufacturer's instructions. As described in the method, a viscometer of type "A" is applicable to the range of viscosity cited in the current work.

Determination of water intake - A sample of about 0.1g of the material to be tested is placed on a microbalance. The sample is dried with a air stream at 25°C of 0% erh (equilibrium relarive humidity) up to no further change in mass is observed (for example less than 0.00005g/min). The mass of the sample is noted.

The sample is then placed at 25°C at 60% erh up to no further change of mass is observed. The amount of water intake is deduced from the change of mass.

Determination of Layer Thickness - Thickness of the layered particle layer may be determined by measuring the d50 of the core particle used prior to coating, and measuring d50 of the core particle after coating. The difference between these two measurements represents the thickness of the layer. Alternatively, SEM analysis can be used to measure the thickness of fractured particles.

Layering Powder Median Particle Size Test - This test method must be used to determine a layering powder's median particle size. The layering powder's particle size test is determined in accordance with ISO 8130-13, "Coating powders - Part 13: Particle size analysis by laser diffraction." A suitable laser diffraction particle size analyzer with a dry-powder feeder can be obtained from Horiba Instruments Incorporated of Irvine, California, U.S.A.; Malvern Instruments Ltd of Worcestershire, UK; Sympatec GmbH of Clausthal-Zellerfeld, Germany; and Beckman-Coulter Incorporated of Fullerton, California, U.S.A.

The results are expressed in accordance with ISO 9276-1:1998, "Representation of results of particle size analysis - Part 1: Graphical Representation", Figure A.4, "Cumulative distribution Q₃ plotted on graph paper with a logarithmic abscissa." The median particle size is defined as the abscissa value at the point where the cumulative distribution (Q₃) is equal to 50 percent.

Determination of Median Particle Size - This test method must be used to determine seed material median particle size.

The particle size test is conducted to determine the median particle size of the subject particle using ASTM D 502 - 89, "Standard Test Method for Particle Size of Soaps and Other Detergents", approved May 26, 1989, with a further specification for sieve sizes used in the analysis. Following section 7, "Procedure using machine-sieving method," a nest of clean dry sieves containing U.S. Standard (ASTM E 11) sieves #8 (2360 um), #12 (1700 um), #16 (1180 um), #20 (850 um), #30 (600 um), #40 (425 um), #50 (300 um), #70 (212 um), #100 (150 um) is required. The prescribed Machine-Sieving Method is used with the above sieve nest. The particle of interest is used as the sample. A suitable sieve-shaking machine can be obtained from W.S. Tyler Company of Mentor, Ohio, U.S.A.

The data are plotted on a semi-log plot with the micron size opening of each sieve plotted against the logarithmic abscissa and the cumulative mass percent (Q₃) plotted against the linear ordinate. An example of the above data representation is given in ISO 9276-1:1998, "Representation of results of particle size analysis - Part 1: Graphical Representation", Figure A.4. The median particle size (D₅₀) is defined as the abscissa value at the point where the cumulative mass percent is equal to 50 percent, and is calculated by a straight line interpolation between the data points directly above (a50) and below (b50) the 50% value using the following equation: ${D}_{50} = {10}^{∧} ⁢ \left[Log\left({D}_{a ⁢ 50}\right)-\left(Log\left({D}_{a ⁢ 50}\right)-Log\left({D}_{b ⁢ 50}\right)\right)*\left({Q}_{a ⁢ 50}-50%\right)/\left({Q}_{a ⁢ 50}-{Q}_{b ⁢ 50}\right)\right]$
where Qₐ₅₀ and Q_{b50} are the cumulative mass percentile values of the data immediately above and below the 50^{th} percentile, respectively; and Dₐ₅₀ and D_{b50} are the micron sieve size values corresponding to these data. In the event that the 50^{th} percentile value falls below the finest sieve size (150 um) or above the coarsest sieve size (2360 um), then additional sieves must be added to the nest following a geometric progression of not greater than 1.5, until the median falls between two measured sieve sizes.

### EXAMPLES

**Example I: Preparation of Co-Particles** - 400 g of sodium percarbonate (SHC from Solvay) is mixed with 64.0 g of maleic acrylic copolymer SOKALAN CP5^{(R)} in Kenwood Food Processor until the mixture is visibly sticky. 200 g of TAED Powder, is then added. Those particles have a thermal stability of 4 microwatts/gram at a Temperature of 40°C after about 48 hours.

**Example II: Preparation of Co-Particles** - 400 g of sodium percarbonate (SHC) is mixed with 56.4 g of maleic acrylic copolymer SOKALAN CP5^{(R)} in a Kenwood Food Processor until the mixture is visibly sticky. 200 g of TAED Powder, is then added with 10g of amorphous silica. Those particles have a thermal stability of 3.5 microwatts/gram at a Temperature of 40 °C after about 48 hours

**Example III: Preparation of Co-Particles (comparative)**- 400 g of sodium percarbonate (SHC) is mixed with 49.0 g of a surfactant mixture comprising 60% of linear alkylbenzene sulphonate and 40% of non ionic surfactant in a Kenwood Food Processor until the mixture is visibly sticky. 200 g of TAED Powder, is then added. Those particles have a thermal stability of 17 microwatts/gram at a Temperature of 40 °C after about 48 hours

The maleic acrylic copolymer is a binder according to the invention absorbing 47.8% of water according to the test method above "determination of water intake" it provides particles (examples I and II) having a better thermal stability than the one having a binder taking less than 5% water according to the test method above "determination of water intake".

The dimensions and values disclosed herein are not to be understood as being strictly limited to the exact numerical values recited. Instead, unless otherwise specified, each such dimension is intended to mean both the recited value and a functionally equivalent range surrounding that value. For example, a dimension disclosed as "40 mm" is intended to mean "about 40 mm."

Every document cited herein, including any cross referenced or related patent or application, is hereby incorporated herein by reference in its entirety unless expressly excluded or otherwise limited. The citation of any document is not an admission that it is prior art with respect to any invention disclosed or claimed herein or that it alone, or in any combination with any other reference or references, teaches, suggests or discloses any such invention. Further, to the extent that any meaning or definition of a term in this document conflicts with any meaning or definition of the same term in a document incorporated by reference, the meaning or definition assigned to that term in this document shall govern.

While particular embodiments of the present invention have been illustrated and described, it would be obvious to those skilled in the art that various other changes and modifications can be made without departing from the spirit and scope of the invention. It is therefore intended to cover in the appended claims all such changes and modifications that are within the scope of this invention.

## Claims

1. A layered particle comprising a core and a layer, said core comprising a source of hydrogen peroxide and said layer comprising a binder and a bleach activator; wherein the weight ratio of said source of hydrogen peroxide to said bleach activator is from about 5:1 to about 1.1:1, or from about 4:1 to about 1.5:1, or about 2:1, and wherein the binder comprises at least 10% by weight of the binder of material absorbing more than 10% water by weight of said binder over a relative humidity of 60% at 25°C.

2. A layered particle according to Claim 1 wherein said binder comprises, based on total binder weight, at least 40% by weight of polymeric material.

3. A layered particle according to any one of the preceding claims wherein said binder comprises, a maleic acrylic polymer, polyvinylpyrolidone, polyethylene glycol or mixtures thereof.

4. A layered particle according to any one of the preceding claims wherein said binder comprises at least 20% by weight of the binder of material absorbing more than 20% water by weight of said binder over a relative humidity of 60% at 25°C.

5. A layered particle according to any one of the preceding claims, wherein said layered particle having a median

6. A layered particle according to any one of the preceding claims wherein said binder comprises, based on total layered particle weight, from about 2% to about 20%, or from about 4% to about 15%, or about 6% to about 10%, or from about 7% to about 8% of said layered particle.

7. A layered particle according to any one of the preceding claims, wherein said binder comprises, based on total layered particle weight, from about 0.001% to about 5%, or from about 0.5% to about 3%, or about 1% to about 2% water.

8. A layered particle according to any one of the preceding claims, wherein said binder is substantially free of water.

9. A layered particle according to to any one of the preceding claims said source of hydrogen peroxide comprising a per-compound, preferably a percarbonate.

10. A layered particle according to to any one of the preceding claims, said bleach activator comprising a material selected from the group consisting of bleach activators such as tetraacetyl ethylene diamine; oxybenzene sulphonate bleach activators such as nonanoyl oxybenzene sulphonate; caprolactam bleach activators; imide bleach activators such as N-nonanoyl-N-methyl acetamide; preformed peracids such as N,N-pthaloylamino peroxycaproic acid, nonylamido peroxyadipic acid, or dibenzoyl peroxide; decanoyloxybenzenecarboxylic acid; and combinations thereof; preferably nonanoyl oxybenzene sulphonate, tetraacetyl ethylene diamine, and combinations thereof, even more preferably tetraacetyl ethylene diamine.

11. A layered particle according to any one of the preceding claims comprising a dusting powder comprising a material selected from the group consisting of silicas; zeolites; amorphous aluminosilicates; clays; starches; celluloses; water soluble salts, preferably an inorganic salt selected from the group consisting of, sodium chloride, sodium sulphate, magnesium sulphate, and salts and mixtures thereof; polysaccharides including sugars; and combinations thereof.

12. A layered particle according to any one of the preceding claims wherein said layer comprises an additive selected from the group consisting of acidic materials, moisture sinks; gelling agents; antioxidants; organic catalyst and combinations thereof.

13. A layered particle according to to claim 12 wherein said additive comprises an acidic material having a pKa of from about 3 to about 7, preferably about 5, preferably ascorbic acid.

14. A layered particle according to Claim 13 wherein said additive comprises a moisture sink selected from the group consisting of crosslinked polyacrylates; sodium salts of maleic/acrylic copolymers; magnesium sulfate; and combinations thereof.

15. A layered particle according to Claim 14 wherein said additive comprises a gelling agent selected from the group consisting of a cellulose including methylcellulose and CMC; alginate and derivatives thereof; starches; polyvinyl alcohols; polyethylene oxide; polyvinylpyrolidone; polysaccharides including chitosan and/or natural gums including carrageenan, xantham gum, guar gum, locust bean gum, and combinations thereof; polyacrylates including cross-linked polyacrylates; alcohol ethoxylates; lignosulfonates; surfactants and mixtures thereof; powdered anionic surfactants; and combinations thereof.
